

July 21, 1959

A. P. LA ROCQUE

2,895,854

METHOD OF MAKING CATHODE ASSEMBLIES AND PRODUCTS

Filed Sept. 28, 1956

2 Sheets-Sheet 1

FIG.1.



FIG.3.



FIG.2.



INVENTOR:  
ARMAND P. LA ROCQUE  
BY

*Hourdon & Hourdon*

ATTYS.

July 21, 1959

A. P. LA ROCQUE

2,895,854

METHOD OF MAKING CATHODE ASSEMBLIES AND PRODUCTS

Filed Sept. 28, 1956

2 Sheets-Sheet 2

FIG. 4.



FIG. 5.



INVENTOR:  
ARMAND P. LA ROCQUE

BY  
*Howson & Howson*  
ATTYS.

1

2,895,854

## METHOD OF MAKING CATHODE ASSEMBLIES AND PRODUCTS

Armand P. La Rocque, Montgomery Township, Pa., assignor to Philco Corporation, Philadelphia, Pa., a corporation of Pennsylvania

Application September 28, 1956, Serial No. 612,670

34 Claims. (Cl. 117—223)

The present invention relates to a novel method for preparing cathode assemblies for electron tubes; and, more particularly, the invention relates to a method for preparing a cathode assembly for electron tubes, such as cathode ray tubes, radio receiving tubes, television receiving tubes, gas discharge tubes, and the like, comprising an oxide-coated cathode and an insulated oxide-coated cathode heater which method provides many important advantages over prior methods. The invention also relates to a cathode assembly, comprising a coated cathode unit and a coated cathode heater unit, from which the ultimate cathode assembly comprising the ultimate oxide-coated cathode and the ultimate insulated oxide-coated cathode heater can be prepared, and to the coated cathode unit and coated cathode heater unit.

The cathode, or "electron emitter," of an electron tube comprises as the cathode unit, a base of nickel containing small amounts of reducing impurities and having a coating of oxides of certain metals, usually of barium and strontium or of barium, strontium and calcium, thereon. In cathode ray tubes the nickel base of the cathode is usually in the form of a cup or cap and the coating is placed on the outside flat surface thereof. In receiving tubes the nickel base is usually in the form of a hollow cylinder and the coating is placed about the periphery thereof extending to within a predetermined distance from the ends of the cylinder. In applying the oxide coating it has been customary practice first to apply to the portion of the nickel base to be coated a suspension of salts of barium and strontium or of barium, strontium and calcium, in a solution of nitrocellulose in an organic vehicle. The vehicle is usually butyl or amyl acetate diluted with acetone or with an alcohol like methanol or amyl alcohol. After the suspension has been applied, the coating is dried and the coated cathode is assembled with the cathode heater, also coated as described below, in cathode assembly form. Electric current is then passed through the heater, generating heat which decomposes the carbonates to oxide form and decomposes the binder.

Much difficulty has been and is being experienced with this procedure. It has been found that coatings applied in this manner often crack, and possess poor adherence to the nickel base. This is particularly true where a dense coating is desired, such as in tubes requiring very close cathode grid spacing, like color television picture tubes. It has been found that this difficulty is due primarily to the sensitivity of the organic system to moisture. It is believed that, during drying of the initial coating, the organic solvents and diluents evaporate rapidly, chilling the air surrounding the coating. This chilling results in condensation of moisture in the air, and the condensed moisture mingles with the nitrocellulose particles in the coating. The binding properties of nitrocellulose are incompatible with the presence of moisture, and when the coating is heated to decompose the salts and to remove the nitrocellulose, the moisture, being converted to steam, expands causing the coating to crack and otherwise disrupting adhesion between the coating and the metal base.

2

This constitutes such a problem in industry, in fact, that resort has been had to the use of vacuum equipment for storage of the cathode bases prior to the application of the coating suspension and the use of air conditioning and humidity control to provide as dry an atmosphere as possible. Such expedients, however, are laborious and expensive, and do not fully eliminate the limitations imposed by such procedure. In addition to the moisture problem, are: the fire and explosion hazard involved with the use of the flammable materials which in turn require the utmost care and expensive equipment; the expense of the solvents and diluents; the harmful effects of the volatile solvents and diluents on workers, and the problem of controlling the purity and composition of the solvents and diluents.

The cathode heater of an electron tube comprises a fine, high-resistance wire, like tungsten, and generally in the form of a helix and having an electrically insulating coating of refractory oxide thereon. In applying the insulating oxide coating it has been customary practice to apply to the high-resistance wire base a suspension of the refractory oxide in a solution of an organic binder in an organic vehicle. After the suspension has been applied, the coating is dried. When the cathode heater and the cathode are assembled and current passed through the heater, the heat decomposes the binder.

Much difficulty has also been experienced with this procedure. It has been found that coatings applied in this manner often chip during handling between drying and the ultimate high temperature heating exposing some of the underlying wire and resulting in short circuiting. The delicate and flexible nature of the wire base thus renders handling so as to avoid damage to the dried coating difficult. In addition to this problem, are: the fire and explosion hazards, the expense of the solvents and diluents; the harmful effects of the volatile solvents and diluents on workers, and the problem of controlling the purity and composition of the solvents and diluents, referred to above in connection with the cathode unit.

It is the principal object of the present invention to provide an improved method for preparing cathode assemblies for electron tubes.

It is another object of the invention to provide an improved method for making electron tube cathode assemblies, involving preparing a carbonate-coated cathode unit and an insulating oxide-coated cathode heater unit, assembling the cathode unit and the cathode heater unit and passing current through the cathode heater unit heating the heater and cathode units including their respective coatings, which method provides substantial advantages over prior methods.

It is another object of the present invention to provide a method for applying the electron emitting oxide coating to a cathode base in the preparation of oxide-coated cathodes for electron tubes whereby cracking and poor adhesion of the coating to the base are eliminated.

Still another object of the present invention is to provide a novel method for preparing oxide-coated cathodes for electron tubes which possess improved operating characteristics over oxide-coated cathodes prepared by previous methods.

It is another object of the present invention to provide a method for applying the electrical-insulating, refractory oxide coating to a cathode heater base in the preparation of oxide-coated cathode heaters for electron tubes whereby chipping and poor adhesion of the coating to the base are substantially reduced.

Still another object of the present invention is to provide a novel method for preparing oxide-coated cathodes and electrical-insulating, refractory oxide-coated cathode heaters whereby fire and explosion hazards are eliminated; fume hazards to workers are removed; problems

concerning the control of purity and composition of solvents and diluents are done away with, and costs, as compared to prior methods, are materially reduced.

Other objects, including the provision of a novel assembly from which the cathode assembly can be prepared, the provision of a novel cathode unit from which the ultimate oxide-coated cathode may be prepared and the provision of a novel cathode heater unit from which the oxide-coated cathode heater may be prepared, will become apparent from a consideration of the following specification and claims.

The method of the present invention comprises applying to the cathode base, a fluid suspension comprising barium and strontium carbonates in an aqueous solution of a water-soluble cellulose derivative selected from the group consisting of salts of carboxymethyl cellulose, carboxymethylhydroxyethyl cellulose and salts of carboxymethylhydroxyethyl cellulose said solution being free of metallic ions known to be detrimental to emission and drying the coating; applying to the cathode heater base, a fluid suspension comprising refractory metal oxide powder in an aqueous solution of a water-soluble cellulose derivative selected from the group consisting of salts of carboxymethyl cellulose, carboxymethylhydroxyethyl cellulose and salts of carboxymethylhydroxyethyl cellulose and drying the coating; assembling the coated cathode and coated cathode heater in cathode assembly form, and passing current through the cathode heater generating heat in the assembly and decomposing the metal carbonates in the cathode coating to oxide form and decomposing the cellulose derivative in both coatings.

The present invention will be more readily understood from a consideration of the drawings in which:

Fig. 1 is an enlarged perspective view, partly in section, of a typical coated cathode for cathode ray tubes;

Fig. 2 is an enlarged perspective view illustrating the step of applying the coating suspension to one end of the cathode base of Figure 1;

Fig. 3 is an enlarged perspective view, partly in section, of a typical coated cathode for receiving tubes;

Fig. 4 is an enlarged perspective view, partly in section, of a typical coated cathode heater; and

Fig. 5 is a vertical sectional view of a cathode assembly showing a cathode heater of the type shown in Fig. 4 mounted in heating relationship within a cathode of the type shown in Fig. 1.

It has been found that the use of a salt of carboxymethyl cellulose or of carboxymethylhydroxyethyl cellulose or carboxymethylhydroxyethyl cellulose itself as binder, in aqueous solution, in the application of the cathode salts to the cathode base and in the application of the insulating, refractory oxide to the cathode heater results in many important unexpected advantages over prior procedures. In the first place, the wet coatings can be dried and baked without danger of cracking. Furthermore, the ultimate oxide coatings are not only free from cracks, but adhere tenaciously to the underlying metal. The coated units thus possess improved handling characteristics so that the danger of chipping or removing a portion of the coating during handling after drying and up to the time they are assembled and heated is materially reduced. By using this procedure, even very dense oxide coatings can be produced, making the procedure especially applicable in the preparation of oxide-coated cathodes for tubes requiring very close cathode grid spacing, such as color television tubes, rectifier tubes having closely spaced elements, and the like. The moisture problem, attending previous procedures for applying the cathode coating, is eliminated by the present procedure. Complicated and expensive expedients, such as vacuum equipment, air-conditioning and dehumidifiers, need not be employed. Because the present method relies upon the use of an aqueous system, the fire and explosion hazards accompanying the previous procedure are eliminated, as are the use of vents and solvent recovery systems, and elec-

trostatic spraying may be used with safety. In addition, it has been found that the carbonate and refractory oxide suspensions are much more stable than the suspensions previously used so that the carbonates and refractory oxides do not settle out, and this is of particular value when automatic spray equipment, such as electrostatic sprayers, is employed. Another important advantage in the use of the present procedure is the ease of control of the purity and composition of the solvent, namely water, inasmuch as distilled water can readily be obtained or produced by those practicing the present process. In this way, careful control of materials entering into the ultimate oxide coating can easily be had. Of course, the aqueous system of the present invention presents no fume hazards to workers, as would the volatile solvents and diluents required by the previous procedures. Finally, water is much less expensive than are the organic solvents and diluents previously required.

One of the more important features of the present invention is the discovery that the ultimate oxide coatings provided on the cathode possess outstanding performance characteristics, that is activity and uniformity of emission, over extended periods of time. This is particularly true when a sodium salt of the cellulose derivative is employed.

The purpose of the process, of course, is to provide an ultimate coating of mixed oxides of barium and strontium, or of barium, strontium and calcium on the cathode base and an electrically insulating coating consisting essentially of refractory oxide on the cathode heater base. Since, in the case of the cathode coating, the oxides are formed in situ through decomposition of carbonates of the stated metals, the suspension initially applied to the cathode base will be a suspension of carbonates of the stated metals. The carbonates are normally in co-precipitated form, such as the so-called "double" carbonate in the case of barium and strontium and the so-called "triple" carbonate in the case of barium, strontium and calcium. The use of the double or triple carbonate results, upon decomposition thereof, in mixed oxide crystals.

In the case of the cathode heater, the suspension initially applied to the cathode heater base will be a suspension of the oxide in powder form. The oxide employed will be such as will be stable and solid at the temperatures to which the heater is subjected during operation, and these may reach 1000-1600° C., depending upon the particular device. A wide variety of metal oxides is available for this purpose, for example, aluminum oxide, zirconium dioxide, magnesium oxide, silicon dioxide, columbium mono- and di-oxides, beryllium oxide, thorium oxide, titanium dioxide, vanadium tri- and tetra-oxides, and the like. Of these, aluminum oxide is preferred.

Referring to the cellulose derivative that is employed as initial binder for the cathode coating and cathode heater coating in accordance with the present invention, it will be, as stated, a water-soluble salt of carboxymethyl cellulose or of carboxymethylhydroxyethyl cellulose or carboxymethylhydroxymethyl cellulose itself. Since, as stated previously, the suspension, especially the suspension applied to the cathode base, will be free of metal ions known to be detrimental to emission, such as zinc, copper, iron, lead, bismuth, chromium, gold, silver, mercury and tin ions, these salts of the cellulose derivatives will not be employed. Other than these, any water-soluble metal, including ammonium, salt of carboxymethyl cellulose or of carboxymethylhydroxyethyl cellulose that either completely decomposes, as does the ammonium salt, or whose metal does not oxidize or whose metal forms a stable oxide at the temperature of the operation of the electron tube, may be employed. Of the metal salts, those of the alkali metals, such as sodium, potassium and lithium, and those of the alkaline earth metals, such as calcium, barium, strontium and magnesium, are preferred. Of these, the sodium salt is particularly advantageous for reasons set forth hereinabove.

Salts of carboxymethyl cellulose are normally prepared

by reacting a salt of cellulose, like sodium cellulose, with an acetate, like sodium monochloracetate. The position for substitution of the carboxymethyl groups is not fixed, and substitution may occur at carbons 2, 3 and/or 6 of the anhydroglucose residues. The degree of substitution is governed by the ratio of acetate to salt of cellulose. Since each anhydroglucose unit in a cellulose molecule contains three reactive hydroxyl groups which can be converted to carboxymethyl groups, theoretically complete reaction would mean the introduction of three carboxymethyl groups per anhydroglucose unit providing a degree of substitution of 3. However, the optimum combination of physical properties are generally achieved with a degree of substitution of from 0.3 to about 1.2, the commercial forms of sodium carboxymethyl cellulose having a degree of substitution of about 0.6-0.9.

Carboxymethylhydroxyethyl cellulose may be prepared by reacting cellulose with a hydroxyethylating agent, such as ethylene oxide, preferably in the presence of caustic alkali, and then reacting the product with a carboxymethylating agent, such as chloracetic acid, preferably in the presence of caustic alkali. The mixed cellulose ether generally contains at least about 0.05 hydroxyethyl group and at least about 0.05 carboxymethyl group for each anhydroglucose unit, and the preferred mixed cellulose ethers contain between about 0.15 and about 0.75 hydroxyethyl group and between about 0.2 and about 0.9 carboxymethyl group for each anhydroglucose unit, the total degree of substitution being at least about 0.50 substituents for each anhydroglucose unit. One commercial form of sodium carboxymethylhydroxyethyl cellulose has an average substitution of 0.3 carboxymethyl groups and 0.7 hydroxyethyl groups, and another commercial form has an average substitution of 0.4 carboxymethyl groups and 0.3 hydroxyethyl groups.

The concentration of cellulose derivative in the aqueous solution is relatively immaterial so long as sufficient is present to hold the carbonate or refractory oxide particles, as the case may be, together to each other and to the respective metal bases until the heating operation is completed, and for this purpose the concentration of cellulose derivative should be at least about 0.5%. Although amounts in excess of 5%, by weight, may be employed, no advantage is gained thereby, and preferably the concentration of cellulose derivative in the solution is between about 0.8 and about 3%, by weight, a concentration of about 1% having been found to be particularly advantageous.

The concentration of the stated cathode metal carbonates or of the refractory oxide in suspension in the respective solutions may vary widely, depending upon the particular means employed for applying the suspension to the cathode and cathode heater bases. For example, when the suspension is applied by dipping, the concentration of the solid particles in the suspension may be very high to the extent where the suspension is in the form of a paste. On the other hand, when the suspension is to be sprayed, the concentration will be relatively low so as to provide a sprayable slurry. With very dilute suspensions, several applications, each of which is followed by drying, may be required.

The relative proportions of the carbonates in the suspension for application to the cathode base may vary somewhat. Generally, the barium carbonate will range between about 30 and about 70 mole percent and the strontium carbonate will range between about 70 and about 30 mole percent, based on the mixture of carbonates. When calcium carbonate is present, it generally will not exceed about 10 mole percent of the mixture of carbonates.

The suspensions may be applied to the respective bases in a wide variety of ways, including dipping, cataphoresis, spraying, and the like. Of these, dipping and cataphoresis are the most common methods for coating the cathode heater base, and spraying is the most common

method for coating the cathode base and in this case a mask may be employed to prevent the suspension from covering those portions of the base to remain uncoated. In this connection, reference may be made to Figure 2 which illustrates one means of application of the suspension to a plurality of cathode bases, for use in cathode ray tubes, by a spraying operation. The numerals 3a represent the cathode bases, 4 represents a mask snugly fitting the ends of the cathode bases, 5 represents the carbonate suspension being directed in spray form toward the upper ends of the cathode bases, 6 represents a conventional spraying device and 7 is a jig for holding the cathode bases during the spraying operation.

After the carbonate suspension has been applied to the cathode base, the coating is dried. This results in a coating comprising the carbonate particles bonded to each other and to the cathode base by means of the cellulose derivative. In this connection, reference may be made to Figures 1 and 3. Figure 1 illustrates a coated cathode base 2 for use in cathode ray tubes. In this case, 1 is the coating and 3 is the base. Figure 3 illustrates a coated cathode base 10 for receiving tubes; 8 being the coating and 9 being the base.

After the refractory oxide suspension has been applied to the cathode heater base, the coating is also dried, resulting in a coating comprising the oxide powder particles bonded to each other and to the cathode heater base by means of the cellulose derivative. In this connection, reference may be made to Figure 4 which illustrates a coated cathode heater base 11, for use in cathode ray tubes. In this case, 13 is the coating and 12 is the base wire.

The coated cathode and coated cathode heater are then mounted in cathode assembly relationship (that is, with the cathode heater in heating relationship to the cathode; normally the cathode heater is mounted within the cathode) in the electron tube assembly. This is illustrated in Fig. 5 where 11 is a coated cathode heater as shown in Fig. 4 inserted within a cathode 2 of the type shown in Fig. 1. The electron tube assembly is evacuated, and current is passed through the cathode heater. This generates heat in the cathode heater base and this in turn heats the cathode heater coating, cathode and cathode coating. Generally the temperature reached in the cathode heater coating is at least 1000° C. and may go as high as 1600° C. and in the cathode coating at least 800° C. and may go as high as 1000° C. The cellulose derivative in both coatings is decomposed and the carbonates in the cathode coating are decomposed to oxide form, the decomposition products being removed, under the vacuum, from the system.

The cathode base, as stated, is generally of nickel or a predominately nickel alloy containing a small amount of a reducing impurity or impurities. Generally, the cathode base will consist of at least 95% of nickel with the remainder being a reducing element or elements like silicon, magnesium, manganese, titanium, tungsten, aluminum and the like. The reducing element or elements activate the cathode causing emission by diffusing through the nickel and reacting with the oxide of the coating to convert the metal oxides to elemental form.

The cathode heater base, as stated, is generally a fine tungsten wire or filament. The diameter of the wire may range from 0.003 to 0.01 inch. Wires or filaments of other high resistance metals capable of generating the required heat upon the passage of current therethrough may be used instead of tungsten, although tungsten is preferred. As also stated, the cathode heater is generally in the form of a helix, as illustrated in the drawing. However, the form of the heater is not critical and depends upon the structure of the particular cathode with which it is used. The cathode heater may be in other forms such as serpentine, loops, spirals or straight.

The present invention will be more readily understood from the consideration of the following specific examples

which are given for the purpose of illustration only and are not intended to limit the scope of the invention in any way.

*Example I*

There are dissolved in 136 cubic cm. of pure distilled water 1.36 grams of sodium carboxymethyl cellulose having a D.S. of 0.65-0.85 and a viscosity in water of 300-600 cps. at 25° C. at 2% concentration (CMC-70 Medium of Hercules Powder Company). To this solution are added 75 grams of the conventional triple carbonate (Ba, Sr and Ca) cathode mix. The mixture is ball milled for about 15 hours. The resulting slurry is then sprayed to one end of a nickel alloy cathode shank ("A-31" alloyed base type of the Superior Tube Company, Norristown, Pa., containing 96% nickel and 4% of tungsten) until a coating .05 mm. thick is built up. The coating is then dried at 25° C. for 12 minutes.

Six cathode units prepared in this manner are subjected to adherence tests in the following manner: Each cathode is mounted, with a cathode heater, on a standard cathode ray stem with a small glass bulb sealed to the stem to complete the assembly. Each cathode is subjected to excessively rapid heating to about 950° C. during which the carbonates are decomposed to oxide form and the cellulose residue decomposed and removed from the coating. In each case the coating remains intact. This is a vigorous test and coatings applied by prior procedures using organic systems generally fail when subjected to this test.

Six more cathodes prepared in this manner were mounted in triode cathode ray tube guns and sealed in 4 inch CR bulbs. The tubes were processed, aged and tested for activity and useful life in the conventional manner with the results listed below:

| Hours..... | 0 | 504 | 720 | 920 | 1,472 | 2,650 |
|------------|---|-----|-----|-----|-------|-------|
|------------|---|-----|-----|-----|-------|-------|

CATHODE ACTIVITY

| Tube:        | 1     | 109   | 109   | 114   | 116              | 101   |
|--------------|-------|-------|-------|-------|------------------|-------|
| 1.....       | 125   | 109   | 105   | 92    | 84               | 118   |
| 2.....       | 120   | 116   | 102   | 110   | ( <sup>1</sup> ) | 117   |
| 3.....       | 110   | 118   | 116   | 119   | 112              | 117   |
| 4.....       | 116   | 122   | 133   | 112   | 106              | 94    |
| 5.....       | 112   | 130   | 123   | 121   | 109              | 118   |
| 6.....       | 106   | 123   | 123   | 114.7 | 105.4            | 109.6 |
| Average..... | 114.7 | 119.7 | 114.7 | 111.3 | 105.4            | 109.6 |

<sup>1</sup> Tube broken on this test.

With this manner of testing, a cathode activity of 80% or better is considered satisfactory. The above results indicate a high degree of emission and good uniformity of activity over a long period of time.

*Example II*

In this example five cathode shanks of "P-50" alloy base of Superior Tube Company (99+% of nickel and traces of the usual reducing impurities) are coated as in Example I. Each of these cathodes is placed in a triode cathode ray gun and sealed in 5 inch CR bulbs, and are processed, aged and tested for activity and useful life with the results given below:

| Hours..... | 0 | 504 | 720 | 920 | 1,472 | 2,650 |
|------------|---|-----|-----|-----|-------|-------|
|------------|---|-----|-----|-----|-------|-------|

CATHODE ACTIVITY

| Tube:        | 1     | 104   | 100 | 80    | 97    | 101   |
|--------------|-------|-------|-----|-------|-------|-------|
| 1.....       | 122   | 92    | 96  | 80    | 108   | 112   |
| 2.....       | 135   | 122   | 84  | 122   | 112   | 124   |
| 3.....       | 125   | 105   | 85  | 101   | 98    | 96    |
| 4.....       | 130   | 123   | 120 | 128   | 119   | 123   |
| Average..... | 128.2 | 109.2 | 97  | 102.2 | 106.8 | 110.8 |

8  
*Example III*

In this example six cathode shanks of the type used in Example II are coated as in Example I using as the coating composition a suspension of 75 grams of the conventional triple carbonate in a solution prepared from 1.36 grams of sodium carboxymethylhydroxyethyl cellulose (average substitution of 0.3 carboxymethyl groups and 0.7 hydroxyethyl groups and a viscosity of 15-100 cps. at a concentration of 2% in water, "CMHEC-37" of the Hercules Powder Company, Wilmington, Delaware). The coating is dried at 25° C. for 12 minutes.

The cathode assemblies are then subjected to adherence tests as in Example I, and in each case the coating remains intact.

*Example IV*

With 260 ccs. of a 1%, by weight, solution of sodium carboxymethyl cellulose having a D.S. of 0.65-0.85 and a viscosity in water of 300-600 cps. at 25° C. at 2% concentration (CMC-70 Medium of Hercules Powder Company) are mixed 140 gms. of fine aluminum oxide powder.

Cathode heater bases of the type illustrated in Fig. 4 of the drawing, the helix of which has an outer diameter of about 0.1 inch and a length of about 0.3 inch and prepared from tungsten wire having a diameter of .0035 inch, are immersed in the resulting suspension and coated by cataphoresis at about 50 volts. The coated heaters are then removed and placed in a gentle stream of air until the coating is dry.

The resulting coated cathode heaters can be subjected to normal handling, which includes welding heater tabs to the lead wires and inserting the heater into the cathode wherein the helix is flexed and compressed, without danger of chipping the coating.

The same procedure is used when applying coating using carboxymethylhydroxyethyl cellulose and its salts as binders.

*Example V*

A coated cathode heater as prepared in Example IV is inserted in a coated cathode as prepared in the first paragraph of Example I. The assembly is mounted in a standard cathode ray tube, the tube evacuated and current is passed through the cathode heater. The heat generated decomposes the sodium carboxymethyl cellulose in both coatings and the carbonate in the cathode coating, the gaseous decomposition products being withdrawn under vacuum. The resulting assembly is ready for use as a cathode ray tube.

Modification is possible in the selection of cellulose derivatives, amounts thereof and constituents of the coatings as well as in the particular techniques followed without departing from the scope of the invention.

I claim:

1. In the preparation of cathode assemblies involving application of a suspension of cathode metal carbonates to a cathode base and drying the coating, application of a suspension of refractory oxide powder to a cathode heater base and drying the coating, assembling the coated cathode heater and cathode in cathode assembly relationship and passing current through the cathode heater to generate heat to heat the assembly, decomposing the coating binders and the carbonates to oxide form, the improvement which comprises applying said carbonates to said cathode base as a suspension in an aqueous solution of a water-soluble cellulose derivative selected from the group consisting of salts of carboxymethyl cellulose, carboxymethylhydroxyethyl cellulose and salts of carboxymethylhydroxyethyl cellulose, said solution being free of metal ions detrimental to emission, and applying said refractory oxide powder as a suspension in an aqueous solution of a water-soluble cellulose derivative selected from the group consisting of salts of carboxy-

methyl cellulose, carboxymethylhydroxyethyl cellulose and salts of carboxymethylhydroxyethyl cellulose.

2. The method of claim 1 wherein the cellulose derivative in each solution is a salt of carboxymethyl cellulose.

3. The method of claim 2 wherein the salt of carboxymethyl cellulose is a sodium salt.

4. In the preparation of oxide-coated cathodes involving application of a suspension of cathode metal carbonates to a cathode base, drying the coating and heating the assembly to decompose the carbonates to oxide form, the improvement comprising applying said carbonates as a suspension in an aqueous solution of a water-soluble cellulose derivative selected from the group consisting of salts of carboxymethyl cellulose, carboxymethylhydroxyethyl cellulose and salts of carboxymethylhydroxyethyl cellulose, said solution being free of metal ions detrimental to emission.

5. The method of claim 4 wherein said cellulose derivative comprises a salt of carboxymethyl cellulose.

6. The method of claim 5 wherein said salt of carboxymethyl cellulose is a sodium salt.

7. The method of claim 4 wherein said cellulose derivative comprises carboxymethylhydroxyethyl cellulose.

8. The method of claim 4 wherein said cellulose derivative comprises a salt of carboxymethylhydroxyethyl cellulose.

9. The method of claim 8 wherein said salt of carboxymethylhydroxyethyl cellulose is a sodium salt.

10. The method of claim 4 wherein the concentration of cellulose derivative in said solution is between about 0.5 and about 5%, by weight.

11. The method of claim 10 wherein the concentration of cellulose derivative is between about 0.8 and about 3%, by weight.

12. The preparation of oxide-coated cathodes which comprises the step of applying to the cathode base a suspension of combined carbonates selected from the group consisting of combined barium and strontium carbonates and combined barium, strontium and magnesium carbonates in an aqueous solution of a water-soluble cellulose derivative selected from the group consisting of salts of carboxymethyl cellulose, carboxymethylhydroxyethyl cellulose and salts of carboxymethylhydroxyethyl cellulose, said solution being free of metal ions detrimental to emission.

13. A cathode unit for electron tubes comprising a cathode base having a coating thereon comprising cathode metal carbonate particles bonded to each other and to the cathode base with a water-soluble cellulose derivative selected from the group consisting of salts of carboxymethyl cellulose, carboxymethylhydroxyethyl cellulose and salts of carboxymethylhydroxyethyl cellulose, said coating being free of metals detrimental to emission.

14. The product of claim 13 wherein said cellulose derivative comprises a salt of carboxymethyl cellulose.

15. The product of claim 14 wherein said salt of carboxymethyl cellulose comprises a sodium salt.

16. The product of claim 13 wherein said cellulose derivative comprises carboxymethylhydroxyethyl cellulose.

17. The product of claim 13 wherein said cellulose derivative comprises a salt of carboxymethylhydroxyethyl cellulose.

18. The product of claim 17 wherein said salt of carboxymethylhydroxyethyl cellulose comprises a sodium salt.

19. In the preparation of oxide-coated cathode heaters involving application of a suspension of refractory oxide powder to a cathode heater base wire and drying the

coating, the improvement comprising applying said oxide powder as a suspension in an aqueous solution of a water-soluble cellulose derivative selected from the group consisting of salts of carboxymethyl cellulose, carboxymethylhydroxyethyl cellulose and salts of carboxymethylhydroxyethyl cellulose.

20. The method of claim 19 wherein said cellulose derivative comprises a salt of carboxymethyl cellulose.

21. The method of claim 20 wherein said salt of carboxymethyl cellulose is a sodium salt.

22. The method of claim 19 wherein said cellulose derivative comprises carboxymethylhydroxyethyl cellulose.

23. The method of claim 19 wherein said cellulose derivative comprises a salt of carboxymethylhydroxyethyl cellulose.

24. The method of claim 23 wherein said salt of carboxymethylhydroxyethyl cellulose is a sodium salt.

25. The method of claim 19 wherein the concentration of cellulose derivative in said solution is between about 0.5 and about 5%, by weight.

26. The method of claim 25 wherein the concentration of cellulose derivative is between about 0.8 and about 3%, by weight.

27. The preparation of oxide-coated cathode heaters which comprises the step of applying to the cathode heater base wire a suspension of aluminum oxide powder in an aqueous solution of a water-soluble cellulose derivative selected from the group consisting of salts of carboxymethyl cellulose, carboxymethylhydroxyethyl cellulose and salts of carboxymethylhydroxyethyl cellulose.

28. A cathode heater unit for electron tubes comprising a cathode heater base wire having a coating thereon comprising refractory oxide powder particles bonded to each other and to the cathode heater base wire with a water-soluble cellulose derivative selected from the group consisting of salts of carboxymethyl cellulose, carboxymethylhydroxyethyl cellulose and salts of carboxymethylhydroxyethyl cellulose.

29. The coated cathode heater unit of claim 28 wherein said coating is free of metals detrimental to emission.

30. The product of claim 29 wherein said cellulose derivative comprises a salt of carboxymethyl cellulose.

31. The product of claim 30 wherein said salt of carboxymethyl cellulose comprises a sodium salt.

32. The product of claim 29 wherein said cellulose derivative comprises carboxymethylhydroxyethyl cellulose.

33. The product of claim 29 wherein said cellulose derivative comprises a salt of carboxymethylhydroxyethyl cellulose.

34. The product of claim 33 wherein said salt of carboxymethylhydroxyethyl cellulose comprises a sodium salt.

#### References Cited in the file of this patent

#### UNITED STATES PATENTS

|           |            |               |
|-----------|------------|---------------|
| 1,739,044 | Ruben      | Dec. 10, 1929 |
| 1,977,318 | McCullough | Oct. 16, 1934 |
| 2,070,816 | Von Wedel  | Feb. 16, 1937 |
| 2,662,028 | Fenton     | Dec. 8, 1953  |

#### FOREIGN PATENTS

|         |               |              |
|---------|---------------|--------------|
| 669,392 | Great Britain | Apr. 2, 1952 |
| 749,429 | Great Britain | May 23, 1956 |

#### OTHER REFERENCES

Hollabaugh et al.: Ind. and Eng. Chem., October 1945, pp. 943-947.

UNITED STATES PATENT OFFICE  
CERTIFICATE OF CORRECTION

Patent No. 2,895,854

July 21, 1959

Armand P. La Rocque

It is hereby certified that error appears in the printed specification of the above numbered patent requiring correction and that the said Letters Patent should read as corrected below.

Column 4, line 57, for "carboxymethylhydroxymethyl" read -- carboxy-  
methylhydroxyethyl --; column 7, line 8, and column 8, line 19, for  
"D.S. of 0.65-0.85", in each occurrence, read -- d.s. of 0.65-0.85 ---.

Signed and sealed this 29th day of March 1960.

(SEAL)

Attest:

KARL H. AXLINE  
Attesting Officer

ROBERT C. WATSON  
Commissioner of Patents